

## UNITED STATES PATENT OFFICE

HUGH S. COOPER, OF CLEVELAND, OHIO, ASSIGNOR TO BERYLLIUM CORPORATION OF AMERICA, OF NEW YORK, N. Y., A CORPORATION OF NEW YORK

## ALLOY AND METHOD OF PREPARING SAME

No Drawing.

Application filed December 2, 1925. Serial No. 72,817.

This invention relates to alloys which have as their chief components silver and beryllium. The main object of the invention is to provide an alloy having special resistance to the action of sulfur compounds. 5 A further object is to reduce the specific gravity of silver in order that it shall possess greater spreading properties. These properties are manifested in alloys containing silver and beryllium and when ductility 10 is also an important consideration, I find that it is desirable to use only rather small amounts of either constituent.

Silver is characterized by its great affinity 15 for sulfur, and the yellow or brownish color which this element quickly assumes in air is due to a film of silver sulfide. The production of a non-tarnishable silver alloy has long been desired.

20 Utilizing beryllium prepared according to my copending application Serial No. 754,446, I have prepared beryllium-silver alloys in nearly all possible compositions. Beryllium is an element which has very little affinity for sulfur, and I have found that even when small percentages of this metal are added to silver or silver alloys, the resistance to tarnishing is increased to an astonishing degree. With only about 3% of 25 beryllium present, the alloys are seemingly immune to vapors of sulfur compounds. Alloys containing about 3% to 5% of beryllium are somewhat brittle in the chill cast condition, but by rolling or otherwise working, at elevated temperatures, and with a final annealing, the various silver-containing compositions within this range are almost as ductile as pure silver.

The great difference in specific gravity of 40 the two metals makes the preparation of uniform alloys somewhat difficult, but I have found that one way of overcoming this difficulty is to first prepare a basic alloy of beryllium and silver, the beryllium content being from 30% to 60%. Such an alloy is 45 very brittle and easily broken into small pieces which can be uniformly mixed. To make the alloy, the silver is first brought into a molten condition under a thin coating 50 of alkali fluoride or chloride flux. Small

proportions of the basic alloy are then added until the desired composition is reached, and when complete solution of the added metal in the silver is effected, the alloy is poured into molds.

55 An alternative method for producing beryllium-silver alloys either in the form of the high-content beryllium basic alloy, or as a directly formed alloy having the desired composition, consists in electrolyzing a beryllium salt with or without an added salt, or salts of more electropositive metals and with or without the addition of beryllium oxide, using molten silver as the cathode.

60 The following will serve as an example: 200 grams of sodium-beryllium fluoride approximating the formula  $2\text{NaF} \cdot \text{BeF}_2$  were melted in a graphite crucible externally heated from  $1100^\circ$  to  $1200^\circ$  C. A carbon anode  $\frac{1}{16}$  of an inch in diameter was 65 immersed to the extent of about 2 inches into the bath. A pool of molten silver at the bottom of the graphite crucible acted as cathode. At intervals additions of beryllium oxide and beryllium fluoride were made. The voltage varied from 5 to 10 volts, the 70 current varying from 15 to 95 amperes.

75 My invention consists not only in the preparation of silver-beryllium alloys but also in the addition of beryllium to technically known silver alloys such as alloys of silver with, for example, aluminum, magnesium, copper, nickel, zinc, cadmium or gold.

80 Alloys having less than about 10% of either silver or beryllium seem at this time preferable because of their better physical properties, but I do not wish to be limited to any specific compositions or proportions except as to those claims which have been 85 purposely and distinctly restricted in this respect.

I claim:

1. An alloy containing substantial amounts up to 10% each of beryllium and silver.
2. An alloy containing silver and from 3% to 5% of beryllium.

95 In testimony whereof, I affix my signature.

HUGH S. COOPER.